

## UNITED STATES PATENT OFFICE

1,959,995

## DYEING PREPARATIONS AND THEIR CONVERSION INTO DYESTUFFS

Arthur Zitscher and Wilhelm Seidenfaden, Offenbach-on-the-Main, Germany, assignors to General Aniline Works, Inc., New York, N. Y., a corporation of Delaware

No Drawing. Application June 16, 1933, Serial No. 676,210. In Germany June 22, 1932

8 Claims. (Cl. 8-6)

The present invention relates to dyeing preparations and to their conversion into dyestuffs.

These dyeing preparations contain an anti-diazo-sulfonate corresponding to the probable general formula:



10 wherein R means an alkyl or aralkyl radical and wherein the benzene nucleus may be substituted by halogen, alkyl or alkoxy, and a combining component containing a hydroxy or an O-alkali-metal group whereof the adjacent position is capable of attaching an arylazo group.

As combining components of the aforesaid kind may be named: 2-hydroxy-naphthalene, its nuclear substitution products as, for instance, aroylamino - hydroxy - naphthalenes, (2 - hydroxy - 20 naphthalene-3-carbonyl)-amino-aryls (as described in U. S. Patents No. 1,101,111 and No. 1,140,747), (6-halogen- or 6-arylamino-2-hydroxy-naphthalene-3-carbonyl)-amino-aryls (see German Patent No. 396,519 and British Patent No. 25 330,349); derivatives of 1-hydroxy-naphthalene-4-carboxylic acid (see U. S. Patent No. 1,453,660) as, for instance, 1-hydroxy-naphthalene-4-phenyl-ketone; compounds containing an acidic methylene group capable of being combined with diazo-compounds as, for instance, pyrazolones and derivatives of beta-ketone-aldehyde, for instance, aceto-acetyl amino-aryls and di-(aceto-acetyl-amino)-aryls (see U. S. Patents No. 1,594,864, No. 30 1,594,866, No. 1,594,867, No. 1,580,709, No. 1,634,-090); dihydroxy-quinolines (see U. S. Patents No. 1,820,039, No. 1,846,073, No. 1,846,074; British Patent No. 332,940); (2-hydroxy-carbazole-3-carbonyl)-amino-aryls, (2-hydroxy-benzocarbazole-3-carbonyl)-amino-aryls, (2-hydroxy-anthracene-3-carbonyl)-amino-aryls.

These dyeing preparations yield when applied in an alkaline medium to fibers, by steaming only, insoluble azo-dyestuffs on the fibers.

Such application to the fiber may consist in dyeing according to the one-bath method, or in printing; the dye-bath or the printing paste, or even the dyeing preparations themselves in powder form, are advantageously mixed with the usual dyeing or printing assistants having wetting, 45 emulsifying or solvent properties, or also with the additional agents customarily used in nitroso-mine-printing colors, such as, for example, chromate.

The anti-diazo-sulfonic acids of the aforesaid 50 constitution may be prepared in the usual man-

ner by transforming the amino group of the corresponding bases into the complex  $-\text{N}=\text{N}-\text{SO}_3\text{H}$ .

The following examples serve to illustrate the invention but they are not intended to limit it thereto, the parts being by weight:

(1) 252 parts of the sodium salt of 4-benzylamino - 2.5 - dimethoxybenzene - 1 - anti - diazo - sulfonic acid of 93% strength (obtainable from 1-amino-4-benzylamino - 2.5 - dimethoxybenzene, yellow powder), 150 parts of 2.3-hydroxynaphthoyl-amino-benzene and 98 parts of anhydrous sodium acetate are ground to form a homogeneous powder. There are obtained 500 parts of dyestuff preparation.

A printing paste which contains 70

|                                              |    |
|----------------------------------------------|----|
| 50 parts of the above dyestuff preparation,  | 70 |
| 20 parts of caustic soda solution of 34° Bé, |    |
| 20 parts of thiodiglycol,                    |    |
| 20 parts of sodium chromate solution 1:4,    | 75 |
| 390 parts of water,                          |    |
| 500 parts of starch tragacanth thickening    |    |

is printed on cotton material; the material is then dried and steamed for 5 minutes in a Mather-Platt apparatus. Thereupon, it is rinsed 30 with an acid solution, soaped and rinsed.

A greenish blue print is obtained.

By using the same anti-diazo sulfonic acid together with 2.3-hydroxynaphthoyl-(1-amino-2-methoxybenzene) and 2.3-hydroxynaphthoyl-(1-amino-4-methoxy-2-methylbenzene), a dark blue print, and by means of diacetoacetyl-4,4'-diamino - 3,3' - dimethyldiphenyl a red-orange print is obtained.

(2) 143 parts of the potassium salt of 4-mono-n-butylamino - 3-chlorobenzene-1-anti - diazosulfonic acid (obtainable from 1-amino-4-mono-n-butylamino-3-chlorobenzene, light-yellow powder), 150 parts of 2.3-hydroxynaphthoyl-(1-amino-2-methyl-5-chlorobenzene) and 207 parts 95 of anhydrous sodium acetate are ground to form a homogeneous powder. There are obtained 500 parts of dyestuff preparation.

A printing paste, prepared from 100

|                                              |     |
|----------------------------------------------|-----|
| 50 parts of the above dyestuff preparation,  | 100 |
| 20 parts of caustic soda solution of 37° Bé, |     |
| 20 parts of thiodiglycol,                    |     |
| 20 parts of sodium chromate solution 1:4,    |     |
| 390 parts of water,                          |     |
| 500 parts of starch tragacanth thickening,   | 105 |

is printed on the material; the material is dried, steamed for 10 minutes in a Mather-Platt apparatus and worked up as usual.

A currant print is thus obtained. 110

By using 2-hydroxycarbazol-3-carbonyl-(1-amino-4-chlorobenzene) and the same anti-diazo sulfonic acid, a brown print is obtained.

(3) 520 parts of the sodium salt of 2.5-dimethoxy-4-(2'4'-dichlorobenzylamino)-benzene-1-anti-diazosulfonic acid of 95% strength, 300 parts of 2.3-hydroxynaphthoyl-(1-amino-3-chlorobenzene), 33 parts of ground sulfur and 147 parts of anhydrous sodium sulfite are ground to form a homogeneous powder. There are obtained 500 parts of dyestuff preparation.

A printing paste prepared from

50 parts of the above dyestuff preparation,  
15 20 parts of caustic soda solution of 37° Bé.,  
20 parts of thioglycol,  
20 parts of sodium chromate solution 1:4,  
390 parts of water,  
500 parts of starch tragacanth thickening,

20 is printed upon the material and the latter is then worked up analogously to Example 1.

A navy blue print is obtained.

(4) 320 parts of a press cake of 69.4% strength from the sodium salt of 2.5-dimethoxy-4-(2'6'-dichlorobenzyl-amino)-benzene-1-anti-diazosulfonic acid, 150 parts of 2.3-hydroxynaphthoyl-(1-amino-4-chlorobenzene) and 105 parts of anhydrous sodium acetate are ground until a dry powder is obtained; thereupon, 25 parts of ground caustic soda are added thereto and the whole is intimately mixed. There are obtained 600 parts of dyestuff preparation.

(5) 250 parts of the sodium salt of 4-methyl-amino-3-chlorobenzene-1-anti-diazosulfonic acid of 88.3% strength, 175 parts of the disodium salt of 2.3-hydroxynaphthoyl-(1-amino-2-methylbenzene) and 75 parts of anhydrous sodium acetate are ground to form a homogeneous powder. There are obtained 500 parts of dyestuff preparation.

40 The process may be applied in the same manner to other kinds of fiber as, for instance, to viscose or to silk.

45 By using other anti-diazosulfonic acids of the aforesaid kind and other azo components, the process may be performed in the same manner.

In the following table we have inserted the shades of a series of further dyeings or prints, produced in an analogous manner:

| 50 | Anti-diazo-sulfonic acid of:                              | Azo-component                                                            | Shade              | 125 |
|----|-----------------------------------------------------------|--------------------------------------------------------------------------|--------------------|-----|
| 1  | 1-amino-4-methylamino-3-chlorobenzene                     | 2.3-hydroxynaphthoyl-(1-amino-2-methylbenzene)                           | Reddish dark blue. |     |
| 2  | Do                                                        | 1-hydroxynaphthalene-4-phenylketone                                      | Brown.             |     |
| 3  | Do                                                        | 2.3-hydroxynaphthoyl-1-aminonaphthalene                                  | Reddish dark blue. |     |
| 4  | 1-amino-4-n-butylamino-3-chlorobenzene                    | 2.3-hydroxynaphthoyl-1-amino-2.5-dimethoxy-benzene                       | Deep garnet.       | 130 |
| 5  | Do                                                        | 2.3-hydroxynaphthoyl-(1-amino-2.5-dimethoxy-4-bromobenzene)              | Bluish garnet.     |     |
| 6  | Do                                                        | 3-methyl-1-phenyl-5-pyrazolone                                           | Reddish yellow.    |     |
| 7  | 1-amino-4-benzylamino-2-methylbenzene                     | 2.3-hydroxynaphthoyl-(1-amino-4-methoxy-3-methylbenzene)                 | Reddish dark blue. |     |
| 8  | 1-amino-4-benzylamino-2-methylbenzene                     | 2-hydroxy-anthracene-3-carbonyl-(1-amino-2-methylbenzene)                | Green-blue.        |     |
| 9  | 1-amino-4-(2'4'-dichlorobenzylamino)-2.5-dimethoxybenzene | 2.3-hydroxynaphthoyl-(1-amino-3-nitrobenzene)                            | Blue.              | 135 |
| 10 | Do                                                        | 6 -bromo - 2.3 - hydroxynaphthoyl - (1 - amino - 2.4 - dimethoxybenzene) | Dark blue.         |     |
| 11 | 1-amino-4-(2'6'-dichlorobenzylamino)-2.5-dimethoxybenzene | 2.3-hydroxynaphthoyl-(1-aminonaphthalene)                                | Greenish blue.     |     |
| 12 | Do                                                        | di-acetoacetyl-4.4'-diamino-3.3'-dimethyldiphenyl                        | Brownish orange.   |     |

70 Since an object of the present invention is to produce dyestuffs of good fastness properties which dyestuffs are insoluble in water and alkalies, it is to be understood that the aromatic nuclei of the general formulæ appearing in the appended claims contain no substituents as are known to render organic compounds soluble in water or alkalies and to tend to deprecate the fastness of the dyestuffs to alkalies. Substituents

of this kind are the sulfonic acid, the carboxylic acid and the hydroxy group.

We claim:

1. As new compositions of matter the dyeing preparations comprising an anti-diazo-sulfonate 80 corresponding to the probable general formula



wherein R means an alkyl or aralkyl radical and wherein the benzene nucleus may be substituted by halogen, alkyl or alkoxy, and a combining component containing a hydroxy or an O-alkali metal group whereof the adjacent position is capable of attaching an arylazo group, which dyeing preparations yield in the presence of caustic alkali by steaming azo-dyestuffs insoluble in water and alkalies. 85

90 2. As new compositions of matter the dyeing preparations comprising an anti-diazo sulfonate corresponding to the probable general formula



95 wherein R means an aralkyl radical and wherein the benzene nucleus may be substituted by halogen, alkyl or alkoxy, and a combining component containing a hydroxy or an O-alkali metal group whereof the adjacent position is capable of attaching an arylazo group, which dyeing preparations yield in the presence of caustic alkali by steaming azo-dyestuffs insoluble in water and alkalies. 100

105 3. As new compositions of matter the dyeing preparations comprising an anti-diazo-sulfonate corresponding to the probable general formula



110 wherein R means a radical of the benzene series, and a combining component containing a hydroxy or an O-alkali metal group whereof the adjacent position is capable of attaching an arylazo group, which dyeing preparations yield in the presence of caustic alkali by steaming azo-dyestuffs insoluble in water and alkalies. 115

120 4. As new compositions of matter the dyeing preparations comprising an anti-diazo-sulfonate corresponding to the probable general formula



125 wherein R means a radical of the benzene series, 145

and a 2,3-hydroxynaphthoyl-amino-aryl, which dyeing preparations yield in the presence of caustic alkali by steaming azo-dyestuffs insoluble in water and alkalies.

5 5. A process which comprises applying to fibers the dyeing preparations claimed in claim 1, drying the fibers, thus applied to, steaming and finishing by rinsing and soaping.

10 6. A process which comprises applying to fibers the dyeing preparations claimed in claim 2, drying the fibers, thus applied to, steaming and finishing by rinsing and soaping.

7. A process which comprises applying to fibers the dyeing preparations claimed in claim 3, drying the fibers, thus applied to, steaming and finishing by rinsing and soaping.

8. A process which comprises applying to fibers the dyeing preparations claimed in claim 4, drying the fibers, thus applied to, steaming and finishing by rinsing and soaping.

ARTHUR ZITSCHER. 85  
WILHELM SEIDENFADEN.

15 90

20 95

25 100

30 105

35 110

40 115

45 120

50 125

55 130

60 135

65 140

70 145

75 150